

## UNITED STATES PATENT OFFICE

2,449,843

## NITRATION PRODUCT OF A HYDROXY AMIDE

William Frederick Filbert, Woodbury, N. J., assignor to E. I. du Pont de Nemours & Company, Wilmington, Del., a corporation of Delaware

No Drawing. Application February 20, 1948,  
Serial No. 9,959

1 Claim. (Cl. 260—467)

1

This invention relates to a new composition of matter and more particularly to a new chemical compound having properties such as to adapt it for use as a commercial explosive.

This is a continuation-in-part of my copending application, U. S. Serial No. 424,903, filed December 30, 1941, now U. S. Patent 2,443,903.

A great many materials and compounds have been proposed for use as explosive charges in detonators or blasting caps. Such compounds may function as base charges, primary charges, or ignition materials. While satisfactory results have been obtained in many respects with the compositions of the prior art, no material or combination of materials has been altogether free from disadvantages.

An object of the present invention is the preparation of a new composition of matter. A further object is a new composition of matter comprising the nitration product of an amide of a hydroxy aliphatic acid. A still further object is a new explosive composition of desirable properties. A further object is a stable explosive composition of relatively high strength. Additional objects will be disclosed as the invention is described more at length hereinafter.

I have found that the foregoing objects are attained by treatment with nitric acid of N-methyl hydroxyacetamide. In this nitration treatment, the addition of nitrogen results from the formation of a nitro group and a nitrate group. The following example will show a specific embodiment of the invention.

2

*Example*

Fifty grams of N-methyl hydroxyacetamide was added gradually to 150 cc. of 98.5%  $HNO_3$  at a temperature below 0° C. Stirring was continued while 150 g. of 96% sulfuric acid was added gradually at such a rate that the temperature did not exceed 50° C. The nitration mixture was then warmed. At 50° C. an active evolution of gas took place. The mixture was cooled and poured into ice water. The creamy white solid separated in the form of small flat rectangular prisms. These were washed with water and purified by gradual dilution of their acetone solution. The material had a melting point of 79–81° C. and showed a nitrogen content of 15.52% when this latter was determined on the nitrometer as against a calculated value for such nitrogen of 15.63% for N-nitro-N-methyl hydroxy acetamide nitrate.

In the foregoing example, nitration has been carried out by means of a sulfuric-nitric mixed acid. In some cases, I may prefer to effect nitration by use of nitric acid and acetic anhydride.

Having described the invention in the preceding, I intend to be limited only by the following claim:

As a new chemical compound, N-nitro-N-methyl hydroxyacetamide nitrate.

30

WILLIAM FREDERICK FILBERT.